

## UNITED STATES PATENT OFFICE.

OTHO V. STEWART, OF WILKINSBURG, AND AUGUST R. HATZFELD, OF TURTLE CREEK, PENNSYLVANIA, ASSIGNORS TO WESTINGHOUSE ELECTRIC & MANUFACTURING COMPANY, A CORPORATION OF PENNSYLVANIA.

## WOOD FILLER.

No Drawing.

Application filed December 16, 1920. Serial No. 431,288.

*To all whom it may concern:*

Be it known that we, OTHO V. STEWART, a citizen of the United States, and a resident of Wilkinsburg, in the county of Allegheny

5 and State of Pennsylvania, and AUGUST R. HATZFELD, a citizen of the United States, and a resident of Turtle Creek, in the county of Allegheny and State of Pennsylvania, have invented a new and useful Improvement 10 in Wood Filler, of which the following is a specification.

This invention relates to a wood filler, and more especially to a composition particularly adapted for filling injured portions 15 and indentations in wood patterns used in casting, it being among the objects of this invention to produce a composition for filling dents and small holes in such patterns, which is cheap, provides a moisture-resistant 20 and strongly adherent mass, and one which hardens very readily.

Wood patterns, such as are used in making molds for casting metal, should have smooth surfaces in order that they may 25 readily be removed from the sand without scarring or mutilating the surface thereof and in order that a smooth casting of the true shape may be formed.

In removing a pattern from the sand, 30 after forming the mold, the molder often taps the same lightly with a hammer in order to more readily release it, thus making indentations in the surface.

Very often, also, nails are driven into a pattern when in the mold, in order that the molder may grasp the same to remove it, especially when the pattern is of large size 35 or is in an awkward position.

Patterns also become damaged accidentally through dropping on a hard floor or 40 being hit by metallic objects of various sorts, and it has been customary hitherto to remove sections of a pattern which became seriously injured and replace the same by 45 new wood. Such an operation is expensive and requires considerable time.

It has also been proposed to fill indentations of small size with putty, paint, iron 50 filler, wood filler, and various other mixtures, but such compositions did not generally become hard, did not adhere permanently to the wood, or left the surface rough.

Our invention obviates these disadvan-

tages and not only results in a coating or filling material which is hard and adherent, 55 but one which may be prepared very readily at small cost.

In practising our invention, we take a viscous solution of shellac or similar material and add to the same a filling material, 60 such as whiting, and form the mixture into a uniform paste. The shellac is usually in an alcoholic solution. The following is a specific example of a mixture which we have found to be suitable for the purpose. 65

Shellac, 3 lbs. 2 ozs.

Denatured alcohol, 1 quart.

Whiting, 6 lbs. 10 $\frac{1}{2}$  ozs.

The shellac is first dissolved in the alcohol, usually with the aid of stirring, 70 after which the whiting is added slowly, with constant stirring, until a uniform, viscous, pasty mass is formed. The mixture is then placed in sealed containers to prevent evaporation of the solvent. This paste may 75 be used for filling wood patterns in substantially the same manner as putty by being worked into place with the aid of a putty knife.

Patterns filled with our material have 80 been subjected to various tests in order to determine the tenacity with which the filler adheres to the wood, and, in all cases, we have found that the pattern may be subjected to very severe conditions without 85 cracking or loss of any of the filler material. The filler in a pattern repaired with my new material has been hammered, and the pattern then immersed in wet sand for several weeks and then baked. Under all these conditions, the filler adhered tenaciously to the 90 wood and was not injured in the least.

Although we have described the use of an alcoholic solution of shellac with whiting as a filling material, it is obvious that various 95 equivalents of shellac, alcohol and whiting may be utilized. For instance, a phenolic condensation product or other natural or artificial resin may be substituted for shellac, acetone or other well-known solvent in place 100 of alcohol, and other inert filling materials, such as lithopone or the like, may be used in place of whiting.

We claim as our invention:

1. A wood filler consisting of shellac and 105 whiting.

2. A wood filler consisting of a viscous solution of shellac and whiting.

3. A wood filler consisting of a solution of three pounds, two ounces shellac and six pounds, ten and one-half ounces whiting.

4. A wood filler consisting of three pounds, two ounces shellac, 1 quart alcohol,

and six pounds, ten and one-half ounces whiting.

In testimony whereof, we have hereunto 10  
subscribed our names this 7th day of December,  
1920.

OTHO V. STEWART.

AUGUST R. HATZFELD.